

# UNITED STATES PATENT OFFICE.

WALTER S. RAVENSCROFT, OF PARKERSBURG, WEST VIRGINIA.

## PULP CASTER-WHEEL.

SPECIFICATION forming part of Letters Patent No. 293,784, dated February 19, 1884.

Application filed April 23, 1883. (No specimens.)

*To all whom it may concern:*

Be it known that I, WALTER S. RAVENSCROFT, a citizen of the United States, residing at Parkersburg, in the county of Wood 5 and State of West Virginia, have invented a new and useful Improvement in Caster-Wheels, of which the following is a specification.

In carrying out my invention, I reduce the paper-pulp or wood fiber to the desirable degree of fineness by any suitable or well-known means, and to a homogeneous mass of a doughy consistence. Chemicals may be added at the proper time to bleach or produce a white article, or coloring-matter may be added and incorporated therewith to give to the mass the proper tint or color. I may also mix with the pulp a suitable proportion of earthy material or resinous substances, or glue may be added, to harden and cause the material to adhere 15 more firmly together. The pulp thus prepared is put into a mold of the desired form and subjected to heavy pressure, the molds being provided with minute apertures, to admit of the escape of water or other moisture 20 when the pulp is formed into the desired shape in a moist or wet condition. The articles, when formed, are taken from the mold, thoroughly dried by any suitable drying medium, and then coated or saturated with boiled linseed-oil or other suitable material, so as to give the 25 article the desired finish. The article is formed with the usual central perforation, to receive

the pin of the castings by which the caster is secured to chairs, tables, &c., as is usual, and a bushing of metal or other suitable material 35 may be secured in the perforation during the process of molding the article or afterward, as may be desired.

I have described the article as made from wet pulp; but I do not wish to limit myself 40 to such, as I may press the pulp in a dry or comparatively dry state into the form desired by subjecting it to sufficient pressure. The pulp may also be mixed with powdered glue or other adhesive material in a dry state, and 45 then subjected to pressure under heat, which will cause the particles to adhere firmly together.

I am aware that it is not new to construct a 50 pulley-wheel of layers or disks of paper or pasteboard forming the web, and other layers surrounding the web to form the rim, the whole being solidified by pressure, and such I do not claim.

Having thus described my invention, what I 55 claim, and desire to secure by Letters Patent, is—

As a new article of manufacture, a caster-wheel made of paper or wood pulp, as set forth.

WALTER S. RAVENSCROFT.

Witnesses:

M. A. BROWN,  
DANE D. JOHNSON.